

## UNITED STATES PATENT OFFICE

2,516,496

AFTERTREATMENT WITH AN ALDEHYDE OF  
WOOL DYED WITH CHROMED AZO DYESWilly Widmer, Bottmingen, and Arthur Buehler,  
Rheinfelden, Switzerland, assignors to Ciba  
Limited, Basel, Switzerland, a Swiss firmNo Drawing. Application October 4, 1948, Serial  
No. 52,793. In Switzerland November 4, 1947

11 Claims. (Cl. 8—43)

1

It is known that in dyeing with metalliferous acid monoazo-dyestuffs, which contain in ortho-position to the azo-linkage an amino group and a hydroxyl group, it is of advantage to carry out the dyeing with the addition of a lower aliphatic aldehyde, especially formaldehyde or a substance yielding formaldehyde. Many dyestuffs of that kind have the undesirable property, even in dyeing in the usual manner from a sulfuric acid bath, but especially with the prolonged dyeing periods, of yielding dull and unsightly dyeings, which is due to decomposition, probably a partial demetallisation of the dyestuff. The prior proposals (see United States Patent No. 2,422,586) state that the aldehyde present in the dyebath has the effect of inhibiting to a great extent the aforesaid decomposition of the dyestuff-metal complex. Obviously this action of inhibiting decomposition can occur only when the formaldehyde or a compound of similar action is present in the dyebath in sufficient quantity during dyeing. As the dyeing process must be conducted at a high temperature (usually at the boil) in order to fix the aforesaid dyestuffs there is a continuous loss of easily volatile formaldehyde, and also considerable difficulties may arise in the dye works due to the odor evolved.

The present invention is based on the unexpected observation that by after-treating with an aldehyde dyeings, which have been produced with acid dyestuffs containing an ortho-amino-ortho'-hydroxy-azo-grouping in the metallized condition, there are obtained results as good as those obtained when an aldehyde is added to the dyebath. There is no obvious explanation for this phenomenon. It can only be supposed that the aldehydes exert a selective decomposing or stripping action on the dyestuff decomposition products formed during the dyeing process, without materially affecting the metal complex proper. However, it is not known that aldehydes can exhibit an action of this kind and it could not be foreseen that they would do so.

As compared with the known process in which the aldehyde must be present in the dyebath in sufficient quantity throughout the whole of the dyeing operation, the process of the present invention has obvious advantages. The present process enables the aldehyde, especially the relatively inexpensive formaldehyde, to be used at a lower temperature or, which is an important advantage, for a shorter period of treatment, and, if desired, in apparatus which is not suitable for dyeing.

There are known a large number of dyestuffs, especially monoazo-dyestuffs and complex metal

compounds thereof, which are suitable for the production of dyeings to be after-treated in accordance with the present invention. For example, they may be derived, on the one hand, 5 from azo compounds capable of coupling in ortho-position to an amino group, especially to 2-amino-naphthalene and sulfonic acids thereof, and, on the other, from ortho-hydroxy-diazo-compounds, care being taken that at least one sulfo group is 10 present in at least one of the two components so that the resulting dyestuff is suitable for dyeing from an acid bath. As coupling components there come into consideration, for example, 2-aminonaphthalene, 2-aminonaphthalene-5- or 15 -6- or -7-sulfonic acid, or 2-aminonaphthalene-3:6- or -5:7-disulfonic acid. As diazo-components there may be mentioned 2-amino-1-hydroxybenzene-4-sulfonic acid, 2-amino-4-chloro-1-hydroxybenzene-6-sulfonic acid, 2-amino-4- 20 methyl-1-hydroxybenzene-5- or -6-sulfonic acid, 2-amino-4- or -5-nitro-1-hydroxybenzene, 2-amino-4-chloro-5- or -6-nitro-1-hydroxybenzene and 2-amino-4:6-dinitro-1-hydroxybenzene.

The dyestuffs obtainable from these components differ in their resistance to decomposition or demetallization so that a small proportion thereof can be used for dyeing without after-treatment with an aldehyde. Those dyestuffs appear to be especially resistant which are derived from ortho-aminophenols containing a sulfonic acid group and a nitro-group. The present invention is of special advantage in the case of dyestuffs derived from nitro-amino-ortho-hydroxybenzenes free from further substituents and 2-aminonaphthalene sulfonic acids. Thus, 30 for example, in the case of dyestuffs from 2-amino-5-nitro-1-hydroxybenzene and 2-amino-naphthalene-5- or -6- or -7-sulfonic acid or 2-amino-naphthalene-5:7- or -3:6-disulfonic acid, and also in the case of dyestuffs derived from 2-amino-1-hydroxybenzene-4-sulfonic acid or 2-amino-4-chloro-1-hydroxybenzene-6-sulfonic acid or 2-amino-4-methyl-1-hydroxybenzene-5- or 40 -6-sulfonic acid and 2-aminonaphthalene.

The dyeings to be after-treated in accordance with the present invention are produced with complex chromium compounds of the foregoing dyestuffs, which have been prepared in substance and contain one atom of chromium per ortho-amino-ortho'-hydroxy-azo-grouping. The dyeing 50 may be carried out in known manner, for example, in the presence of 4-8 per cent. of sulfuric acid (calculated on the fiber to be dyed) and at boiling temperature if desired with the addition of a salt such as sodium sulfate.

For after-treating such dyeings in accordance

with the present invention a very wide variety of aldehydes may be used. There may be mentioned principally lower aliphatic aldehydes such as acetaldehyde, especially formaldehyde. The aldehydes may be used either as such or in the form of an ordinary commercial aqueous solution or in the form of polymerization or condensation products yielding the aldehyde. In the latter connection there may be mentioned polymerized acetaldehyde, paraformaldehyde, condensation products of amines or phenols with formaldehyde which contain the formaldehyde in loose combination such as melamine-formaldehyde condensation products or urea-formaldehyde condensation products having a high content of formaldehyde.

There also come into consideration aldehydes which are derived from organic radicals of high molecular weight and contain the aldehyde group bound to a heterocyclic or carbocyclic, advantageously aromatic, ring such as furfural, phthalaldehyde, salicylaldehyde, and the like. Furthermore, in some cases there may be used with advantage aldehydes which contain besides the aldehyde group at least one ionisable acid group, such as benzaldehyde mono- or di-sulfonic acids or mono- or di-carboxylic acids. As examples there may be mentioned benzaldehyde-2- or -3- or -4-sulfonic acid, 4-nitro-benzaldehyde-2-sulfonic acid and benzaldehyde-2:4- or -2:5-disulfonic acid, and also benzaldehyde-2- or -3- or -4-carboxylic acid. There are also suitable for the present invention aldehydes which, owing to the presence of a basic group, are capable of forming water-soluble salts with mineral acids, especially sulfuric acid. 3-aminobenzaldehyde is an example of such an aldehyde.

The after-treatment of the aforesaid dyeings may be applied at any time after the whole or at least the greater part of the dyeing process has been carried out. The after-treatment may therefore be carried out in the dyebath itself, if desired after it has cooled somewhat, or in a fresh bath with or without intermediate drying of the material. By the use of a fresh bath the after-treatment bath can be maintained acid, and advantageously strongly acid, by the addition of an acid, for example, sulfuric acid.

The proportion of the aldehyde to be used in the after-treatment of this invention may vary within wide limits, since a small addition of about 0.5 per cent. generally has a certain effect and large additions of about 10 or more percent. do not as a rule have a deleterious effect. In many cases an addition of 1-6 per cent. of formaldehyde or 2-8 per cent. of a benzaldehyde sulfonic acid is of advantage.

The after-treatment may be conducted in an aqueous bath at a moderately raised temperature, for example, about 40-50° C., for a period ranging from one to several hours. At higher temperatures in the region of 90-100° C. considerably shorter periods of treatment give the result, for example, a period of treatment of 15 minutes.

In the case of easily volatile aldehydes such as formaldehyde or benzaldehyde, the after-treatment may also be carried out by subjecting the dyed and, if desired, dried material for a long time to the action of the vapor of the aldehyde. Provided that the period of treatment is sufficiently long this method of after-treatment leads to a quite substantial improvement in the dyeing even when it is carried out at room temperature. In order to avoid losses of aldehyde and troubles due to odors the process is advantageously carried out in a closed space (a steam chamber).

The following examples illustrate the invention, the parts being by weight:

*Example 1*

100 parts of wool are dyed in the usual manner with 1.5 parts of the complex chromium compound of the dyestuff from diazotized 5-nitro-2-amino-1-hydroxybenzene and 2-amino-naphthalene-6-sulfonic acid from a dyebath which contains 8 parts of sulfuric acid and 10 parts of crystalline sodium sulfate. When the dyeing is finished there are added to the hot dyebath at 98-100° C. 5 parts of an aqueous formaldehyde solution of 40 per cent. strength and the bath is maintained at 98-100° C. for a further 15 minutes. The wool is then rinsed and finished in the usual manner. A level pure yellowish green dyeing is obtained.

By using instead of formaldehyde 2 parts of para-formaldehyde or 5 parts of a water-soluble condensation product of formaldehyde and melamine, there is likewise obtained a pure yellowish green wool dyeing.

*Example 2*

100 parts of wool are dyed as described in Example 1 with 1.5 parts of the complex chromium compound of the dyestuff from diazotized 5-nitro-2-amino-1-hydroxybenzene and 2-amino-naphthalene-6-sulfonic acid. When the dyeing is finished there are added to the hot dyebath at 98-100° C. 5 parts of benzaldehyde-3-sulfonic acid and the aldehyde sulfonic acid is allowed to act for one hour at 100-90° C. Then the wool is rinsed and finished in the usual manner. There is obtained a green wool dyeing which is substantially purer and of a more yellow shade than that which is obtained without after-treatment with benzaldehyde-3-sulfonic acid.

*Example 3*

100 parts of wool are dyed in the usual manner with 1.5 parts of the complex chromium compound of the dyestuff from diazotized 4-chloro-2-amino-1-hydroxybenzene-6-sulfonic acid and 2-aminonaphthalene from a dyebath which contains 8 parts of sulfuric acid and 10 parts of crystalline sodium sulfate. When the dyeing is finished there is added to the hot dyebath at 98-100° C. 1 part of formaldehyde and the bath is maintained at that temperature for one hour. The wool is then rinsed and finished. It is dyed a level, pure, blue-green tint. Without the after-treatment with formaldehyde the dyeing would be considerably duller.

*Example 4*

100 parts of wool are dyed in the manner described in Example 1 with 1.5 parts of the complex chromium compound of the dyestuff from diazotized 5-nitro-2-amino-1-hydroxybenzene and 2-aminonaphthalene-6-sulfonic acid. When the dyeing is finished the wool is rinsed and entered into a fresh bath at 60-70° C. This fresh bath is mixed with the dilute sulfuric acid solution of benzaldehyde-3-sulfonic acid, which contains 1 part of the said sulfonic acid and 8 parts of sulfuric acid. The bath is slowly raised to the boil and then maintained at 98-100° C. for 1 hour. The wool is then rinsed and finished in the usual manner. It is dyed a uniform pure yellowish green tint. Without the after-treatment with benzaldehyde-3-sulfonic acid a considerably bluer and duller dyeing would be obtained.

Instead of the sulfuric acid solution of benzaldehyde-3-sulfonic acid, there may be added to

the after-treatment bath a solution of 1.5 parts of 3-aminobenzaldehyde in 80 parts of sulfuric acid of 10 per cent. strength, the procedure being the same in other respects. In this case also a pure yellowish green dyeing is obtained.

*Example 5*

100 parts of wool are dyed in the manner described in Example 1 with 1.5 parts of the complex chromium compound of the dyestuff from diazotized 5-nitro-2-amino-1-hydroxybenzene and 2-aminonaphthalene-6-sulfonic acid. When the dyeing is finished the wool is rinsed and dried. The wool so dyed is suspended in a closed chamber at room temperature. The closed chamber is saturated with formaldehyde vapor. This is brought about by inserting in the lowest part of the chamber, (for example in a flat dish) an aqueous solution of formaldehyde of 40 per cent. strength. The wool should not come into contact with the formaldehyde solution. The wool is kept in the chamber at room temperature for 18 hours. At the end of this period the previously bluish, dull dyeing is a pure yellowish green.

Similar results are obtained by suspending for 18 hours in a closed chamber over a formaldehyde solution, instead of dry wool, moist wool, for example as it is obtained after dyeing and rinsing. Instead of formaldehyde solution ordinary commercial benzaldehyde may be used for the treatment of the moist wool, the action of benzaldehyde on dry wool being considerably slower.

What we claim is:

1. A process for after-treating dyeings produced on wool with acid dyestuffs containing an ortho-amino-ortho'-hydroxy-azo-grouping in the chromed condition, wherein the dyeing is treated with an aldehyde.

2. A process for after-treating dyeings produced on wool with acid dyestuffs containing an ortho-amino-ortho'-hydroxy-azo grouping in the chromed condition, wherein the dyeing is treated with a lower aliphatic aldehyde.

3. A process for after-treating dyeings produced on wool with acid dyestuffs containing an ortho-amino-ortho'-hydroxy-azo grouping in the chromed condition, wherein the dyeing is treated with a lower aliphatic aldehyde which is used in the form of a condensation product or polymerization product capable of yielding said aldehyde.

4. A process for after-treating dyeings produced on wool with acid dyestuffs containing an ortho-amino-ortho'-hydroxy-azo grouping in the chromed condition, wherein the dyeing is treated with formaldehyde.

5. A process for after-treating dyeings produced on wool with acid dyestuffs containing an ortho-amino-ortho'-hydroxy-azo grouping in the chromed condition, wherein the dyeing is treated with formaldehyde which is used in the form of a condensation or polymerisation product capable of yielding formaldehyde.

6. A process for after-treating dyeings produced on wool with acid dyestuffs containing an ortho-amino-ortho'-hydroxy-azo grouping in the chromed condition, wherein the dyeing is treated with an aldehyde containing an ionisable acid group.

7. A process for after-treating dyeings produced on wool with acid dyestuffs containing an ortho-amino-ortho'-hydroxy-azo grouping in the chromed condition, wherein the dyeing is treated with an aromatic aldehyde sulfonic acid.

8. A process for after-treating dyeings produced on wool with acid dyestuffs containing an ortho-amino-ortho'-hydroxy-azo grouping in the chromed condition, wherein the dyeing is treated with a benzaldehyde sulfonic acid.

9. A process for after-treating dyeings produced on wool with acid dyestuffs containing an ortho-amino-ortho'-hydroxy-azo grouping in the chromed condition, wherein the dyeing is treated with benzaldehyde-3-sulfonic acid.

10. A process for after-treating dyeings produced on wool with acid dyestuffs containing an ortho-amino-ortho'-hydroxy-azo grouping in the chromed condition, wherein the dyeing is treated with a mineral acid salt of an aldehyde containing a basic group.

11. A process for after-treating dyeings produced on wool with acid dyestuffs containing an ortho-amino-ortho'-hydroxy-azo grouping in the chromed condition, wherein the dyeing is treated with sulfate of 3-aminobenzaldehyde.

40 WILLY WIDMER.  
ARTHUR BUEHLER.

REFERENCES CITED

The following references are of record in the file of this patent:

UNITED STATES PATENTS

| Number    | Name   | Date          |
|-----------|--------|---------------|
| 2,263,894 | Sparks | Nov. 25, 1941 |
| 2,422,586 | Royer  | June 17, 1947 |

FOREIGN PATENTS

| Number  | Country | Date          |
|---------|---------|---------------|
| 502,314 | France  | Feb. 19, 1920 |
| 596,888 | Germany | May 12, 1934  |